

## UNITED STATES PATENT OFFICE

CLARENCE W. BALKE, OF HIGHLAND PARK, ILLINOIS, ASSIGNOR TO FANSTEEL PRODUCTS COMPANY, INC., OF NORTH CHICAGO, ILLINOIS, A CORPORATION OF NEW YORK

## PROCESS FOR OBTAINING METALLIC TANTALUM

No Drawing.

Application filed August 20, 1923. Serial No. 658,289.

This invention relates to the method or process of obtaining substantially pure metallic tantalum.

The object of this invention is to provide a process by which substantially pure metallic tantalum in a workable form may be obtained by a comparatively few steps which may be readily carried out.

Briefly stated, the first step in the process 10 consists in electrolyzing a fused salt of tantalum containing a dissolved oxide of tantalum, using a carbon (preferably graphite) electrode. It has been found convenient to carry out the electrolyzing process in a furnace consisting of an iron pot which constitutes the cathode, the anode being a relatively large rod of graphite. A rod four or 15 five inches in diameter has been found satisfactory.

20 In carrying out the present process the double salt of tantalum, potassium fluotantalate ( $K_2TaF_7$ ), and tantalic oxide ( $Ta_2O_5$ ) are employed. Preliminary to the electrolyzing process it has been found desirable to 25 fuse or melt a portion of the double fluoride. After the double fluoride has become fused, the oxide is added and readily dissolves. The electrolysis is then carried out by passing direct current through the furnace.

30 It has been found that the double fluoride may be conveniently fused by using an auxiliary graphite electrode and employing alternating current. Thus a portion of the double fluoride will first be placed in an iron 35 pot and fused by alternating current and the auxiliary electrode as just stated. As soon as a sufficient quantity of the double fluoride has become fused, a small quantity of the oxide is added and the electrolysis is started 40 by passing direct current through the furnace, the auxiliary electrode being no longer employed.

During the electrolysis the tantalum is 45 produced in the form of crystals which deposit in the pot, building up a sponge-like mass which consists of a mixture of these crystals with tantalum salt. As the mass builds up, the graphite electrode is gradually raised. The electrolysis is continued 50 with the addition, from time to time, of salt

and oxide until the pot has become filled, or a sufficient quantity deposited therein, when the mass is permitted to solidify.

This product of electrolysis is a grey or sometimes black mass, consisting largely of 55 the double fluoride of tantalum, some oxide and the metallic crystals above referred to. The mass also contains more or less graphite which has sloughed off during the electrolysis process. Part of the anode which has disappeared during the electrolyzing process has united with the oxygen of the oxide and passed off as carbon monoxide or perhaps, the dioxide. If the electrolysis process has been properly carried out, the mass remaining in the pot at the end of the process will contain in the neighborhood of fifteen per cent (15%) of metallic tantalum. The mass shrinks upon cooling and may be readily removed from the pot.

50 After the mass has cooled, it is ground to a fine powder. This grinding process acts to a great extent to free the metal crystals from the salt with which the crystals are mechanically combined in the product of the electrolysis.

The grinding process may be very conveniently carried out by passing the material through an impact pulverizer, using air separation. By this means the bulk of the 80 salt is removed from the metal crystals. The metal crystals may be further purified by passing the mass over a Wilfley table or by decantation. When run over the Wilfley 85 table the metal crystals which are deposited at one end of the table will be found to be almost pure. The material at the other end of the Wilfley table will be found to be largely salt, while the intermediate portion will contain both salt and metal crystals. In certain cases it may be found desirable to treat 90 the impure metallic powder by passing it over the Wilfley table and also by decantation. It is found that the decantation process is particularly desirable in removing the loose 95 graphite particles from the powder.

The metallic powder, containing more or less impurities according to the position on the table where it is delivered, may be treated 100 chemically to assist in purifying it. My

process is to treat it alternately with a solution of potassium hydroxide and dilute hydrofluoric acid. Sometimes treatment with dilute aqua regia has a beneficial result.

5 This process partly dissolves the salt and partly loosens it from the metallic particles so that a few treatments with washing and decantation of the lighter material will leave the metal free from all of the salt and most 10 of the carbon. In certain instances it may be found preferable to treat the impure metal powder with the hydroxide and acid and employ the Wilfley table last as a means for further reducing the amount of graphite remaining mixed with the metal powder. In 15 other instances it may be found desirable to employ the Wilfley table both before and after treating the powder with chemicals.

The chemically treated powder is found 20 to be practically entirely free from salt and to contain less than one-half of one-percent of carbon. By the use of the Wilfley table the carbon content may be reduced to one-tenth of one-percent, or, in some cases, very much lower. It is to be understood that the order 25 of the steps, and in fact the entire manner of mechanically separating the metal particles from the rest of the mass may be greatly varied and still get good results. The 30 method above described has, however, been found to be very satisfactory.

The process thus far described has resulted 35 in producing a metallic powder of tantalum which is substantially chemically pure and which has mechanically mixed with it a very small fraction of carbon. When the process has been properly carried out as above explained, the carbon remaining in the powder is reduced to less than one-tenth of one- 40 per cent.

Practically pure powder may be obtained by double electrolysis. In carrying out the second process of the electrolysis a crude tantalum bar may be employed as the anode. 45 It has been found, however, that the anode bar disappears very rapidly during the electrolysis and the amount of metal obtained from the electrolysis does not exceed, and generally is much less than, the amount lost from the anode. Therefore, this process is 50 not desirable and should be used only when it is essential that an absolutely pure tantalum be secured.

In order to obtain a homogeneous bar of 55 tantalum from tantalum powder, the powder is pressed into a bar and is then sintered in a vacuum furnace. In pressing the bar it is desirable to use as high a pressure as possible as the metal grains are relatively coarse, and 60 it has been found that high pressure actually causes the metal grains to flow more or less in the die and a very compactly pressed bar is thus obtained.

After the pressed bar has been formed, it 65 is placed in the furnace and clamped between

the upper and lower electrodes of tungsten or molybdenum. One of the electrodes of the furnace must be movable as the bar contracts during the sintering process. The furnace is assembled and exhausted with a suitable air pump and the current turned on and maintained on until the vacuum suddenly drops.

This first drop in vacuum is probably 70 caused by moisture in the bar which is driven out when the bar is heated. It may be due, in part at least, to occluded gas. To obtain the most satisfactory result, the current is flashed on in this manner two or three times until the drop in vacuum is not great.

The current is now left on at a relatively 75 low amperage, in the neighborhood of eight-hundred amperes for a three-eighths inch square pressed bar, until a vacuum is reached of about one-tenth to two-tenths of a millimeter of mercury. The current used will, of course, vary with the cross sectional area of the pressed bar. The current is now gradually increased until the bar is heated substantially to its melting point, or probably to 80 about 2700°-2800°. In short, the bar is heated as hot as it safely can be without danger of melting the core of the bar. The bar is maintained at the high temperature until the vacuum comes back to about one-tenth to two-tenths of a millimeter of mercury, when the current is turned off. This 85 process may take one-half to three-quarters of an hour, or it may take much longer. For the three-eighths inch square bar, a current of nearly two-thousand amperes is usually required to bring the bar to the necessary high temperature. A bar one-half inch by five-eighths inch requires a current of about 90 twenty-eight hundred amperes.

100 During the sintering process, every increase in temperature causes a further drop in vacuum until, near the end of the sintering process, the vacuum comes back. This is probably due to the bar giving up the gas 105 therein.

The sintered bar thus formed is a homogeneous piece of metal, similar in shape to the pressed bar, but somewhat shorter and is suitable for rolling or swaging cold. Most of the free carbon remaining mixed with the metal particles forming the pressed bar passes away during the sintering process, particularly if a small amount of tantalum 115 oxide is added to the metal powder of which the bar is formed.

120 While in the above description my approved process is described, it is to be understood that this process may be varied slightly in some particulars and still obtain satisfactory results. The invention, therefore, is to be limited merely by the scope of the hereunto appended claims.

125 Having now described my invention, what 130

I claim as new and desire to secure by Letters Patent of the United States, is:

1. The process of obtaining tantalum which comprises electrolyzing a fused bath containing tantalic oxide and potassium fluotantalate.
2. The process of obtaining tantalum which comprises fusing potassium fluotantalate, adding tantalic oxide to the fused salt, and electrolyzing the fused mass.
3. The process of obtaining tantalum which comprises electrolyzing a fused bath of potassium tantalum fluoride and replacing the tantalum removed from the fused bath by adding a tantalum oxide which is soluble in the potassium tantalum fluoride.
4. A process of obtaining tantalum which comprises electrolyzing a fused bath of potassium fluotantalate and tantalic oxide, pulverizing the products of the electrolysis, mechanically removing the powder from the rest of the mass and alternately treating said powder with potassium hydroxide and an acid.
5. A process of producing workable bodies of tantalum which comprises electrolytically preparing granules of metallic tantalum from a fused bath of potassium tantalum fluoride and a tantalum oxide dissolved therein, mechanically and chemically separating said granules from the products of the electrolysis, forming said granules into a body of the desired size and shape and removing the carbon impurities from said body by sintering.

In witness whereof, I hereunto subscribe my name this 17th day of August, 1923.

CLARENCE W. BALKE.

40

45

50

55

60

65